

**1**

3,378,916

**MANUFACTURE OF SUPERCONDUCTING WIRE**  
Peter Robinson, Fossway, Newcastle-upon-Tyne, England,  
assignor to International Research & Development  
Company Limited, Fossway, Newcastle-upon-Tyne,  
England

No Drawing. Filed Oct. 21, 1965, Ser. No. 500,218  
Claims priority, application Great Britain, Oct. 30, 1964,  
44,416/64

2 Claims. (Cl. 29—599)

The present invention relates to processes for the production of superconducting niobium-zirconium alloy wire.

Niobium-zirconium alloys, in the form in which they are normally obtained, are relatively brittle and difficult to fabricate into wire. This is particularly true of alloys with high oxygen, carbon, hydrogen and nitrogen contents.

The present invention provides a process in which the material is subjected to a series of treatments to overcome these difficulties and to produce niobium-zirconium alloy wire of improved superconducting properties.

It is necessary to start with a material having a refined crystal structure, that is to say, a material in which dendritic crystal structure and high concentrations of impurities are substantially absent. When the material has been formed by casting, the as-cast structure should be broken down by mechanical working, preferably hot working. When the material has been formed by powder metallurgy techniques, the amount of working necessary to produce a refined crystal structure may be considerably less.

The process in accordance with the invention for the production of superconducting niobium-zirconium alloy wire comprises the following steps:

(1) Heat-treating a niobium-zirconium material having a refined crystal structure as herein defined, in a temperature range 1000°—1250° C. under inert conditions for 30—120 minutes.

(2) Quenching the material as quickly as possible to retain the second phase constituents in solution.

(3) Working the material at a temperature below 500° C. to reduce its cross-section and removing any surface defects which may be present.

(4) Further heat-treating the material at a temperature in the range 750° C.—825° C. under inert conditions for 15—130 minutes.

(5) Enclosing the material in a sheath of different material having substantially similar working properties to the material regarding ductility, rate of work-hardening and hardness.

(6) Deforming the material and sheath together to the required final cross-section of the material.

(7) Dissolving the sheath.

(8) Copper-plating the material.

The material of the sheath may be "Inconel" alloy. The copper-plating step preferably includes hydriding the material and depositing a film of nickel before the copper is deposited.

The process will now be described in more detail with the aid of an example. A cast ingot of niobium-zirconium was used having the analysis by weight: Zirconium 27.8%, balance niobium, oxygen 74 parts per million, nitrogen 50 parts per million, carbon 125 parts per million and hydrogen 2 parts per million. The ingot was hot-extruded to a diameter of  $\frac{3}{4}$ " to break down the as-cast structure and then heat-treated at 1200° C. for one hour in an atmosphere of static inert gas, for example, argon, or in vacuum. The heat treatment was carried out in a metal canister, for example, of mild steel protected against oxidation by a refractory frit and the whole subsequently quenched in water at room temperature (about 15° C.).

**2**

The heat-treated ingot was then cold swaged at room temperature to 0.110 inch diameter rod and dressed, for example, by grinding and filing, to remove any surface defects. It was then given further heat treatment at 800° C. for fifteen minutes in a static argon atmosphere. This treatment was carried out in an argon-filled copper tube which was a loose fit on the rod. The ends of the tube were sealed by high-temperature brazing. The canned rod was passed continuously through a furnace to give the desired heat treatment.

After removal from the copper can the rod was placed in a cold drawn "Inconel" tube 0.160 outer diameter and 0.130 inner diameter. One end of the tube was swaged on to the rod and the tube then drawn tightly on to the rod. The composite member was then cold drawn until the diameter of the wire forming the core of the composite member was 0.010 inch.

The "Inconel" sheath was then dissolved off the rod by an electrolytic process by a batch technique using a solution of 5% sulphuric acid at 2.3 volts potential difference.

Finally, the wire was plated using a continuous process apparatus such as is described in our copending application No. 27,614/64. The wire was first degreased then etched in 10% hydrofluoric acid solution at 38° C. and then hydrided electrolytically in 2% hydrofluoric acid (cold) at a current density of 40 amps. per square foot.

A nickel flash plating 0.0001 inch thick was then given to the wire at a current density of 40 amps. per square foot and finally copper was deposited from an acid sulphate bath at a current density of 140 amps. per square foot to give a final overall plating thickness on the wire of 0.001 inch.

In the casting of the niobium-zirconium alloy the second phase constituents, that is to say, oxygen, carbon, hydrogen and nitrogen, are preferentially precipitated at the grain boundaries, resulting in embrittlement of the material. After extrusion of the ingot to break down the as-cast structure, the first heat treatment produces solution of the second phase constituents and the quenching retains most of the second phase constituents in solution. Any second phase constituents which are precipitated during the quenching are dispersed throughout the material and are thus less harmful. The resulting reduction in embrittlement means that alloys with high oxygen, carbon, hydrogen and nitrogen contents can be fabricated. The ease of fabrication can be estimated by measuring the hardness of the material before and after the initial heat treatment. It is found that the alloy can be more easily fabricated if its hardness before the heat treatment is below 265 VPN (Vickers Pyramid Number) and is not increased by the treatment.

The initial heat treatment followed by cold working and subsequent thermal precipitation treatment (Step 4) has a beneficial effect on the superconducting properties of the material.

The process can be used to advantage from the points of view of fabrication and improvement of superconducting properties with most niobium-zirconium alloys.

In the example described above the working of the material after the first heat treatment took place at room temperature, but this working can be carried out at temperatures up to about 500° C.

Materials other than "Inconel" can be used for the enclosing sheath providing they have properties similar to those of the niobium-zirconium alloy regarding ductility, rate of work-hardening and hardness. The purpose of the sheath is to reduce the effect of galling between the wire and the die through which the wire is drawn.

I claim:

1. A method or process for the production of super-

conducting niobium-zirconium alloy wire comprising the following steps:

- (a) heat-treating a niobium-zirconium material containing a second phase constituent and having a substantially non-dendritic refined crystal structure substantially free of high concentrations of impurities, in a temperature range 1000°-1250° C. under inert conditions for 30-120 minutes, whereby said second phase is placed in solution with said material;
- (b) quenching the material as quickly as possible to retain the second-phase constituents in solution;
- (c) working the material at a temperature below 500° C. to reduce its cross section and removing any surface defects which may be present;
- (d) further heat-treating the material at a temperature in the range 750° C.-825° C. under inert conditions for 15-130 minutes;
- (e) enclosing the material in a sheath of different material having substantially similar working properties to the material regarding ductility, rate of work-hardening and hardness;

(f) deforming the material and sheath together to the required final cross-section of the material;

(g) dissolving the sheath;

(h) copper-plating the material.

- 5 2. A process as claimed in claim 1 in which the copper-plating step includes hydriding the material and depositing a film of nickel before the copper is deposited.

#### References Cited

##### UNITED STATES PATENTS

|           |         |               |       |        |
|-----------|---------|---------------|-------|--------|
| 3,109,963 | 11/1963 | Geballe       | ----- | 29—599 |
| 3,131,469 | 5/1964  | Glaze.        |       |        |
| 3,204,326 | 9/1965  | Granitas.     |       |        |
| 3,218,693 | 11/1965 | Allen et al.  | ----- | 29—599 |
| 3,239,919 | 3/1966  | Levi.         |       |        |
| 3,277,564 | 10/1966 | Webber et al. | ----- | 29—419 |

JOHN F. CAMPBELL, *Primary Examiner.*

PAUL M. COHEN, *Assistant Examiner.*